

E. WEINTRAUB,  
ELECTRICAL HEATING DEVICE,  
APPLICATION FILED OCT. 16, 1913.

1,118,387.

Patented Nov. 24, 1914.

Fig.1.



Fig.2.



Fig.3.



Fig.4.



Witnesses:

Marcus L. Byng.  
J. Ellis Elmer

Inventor:  
Ezechiel Weintraub,  
by *Alfred, Davis*  
His Attorney.

# UNITED STATES PATENT OFFICE.

EZECHIEL WEINTRAUB, OF LYNN, MASSACHUSETTS, ASSIGNOR TO GENERAL ELECTRIC COMPANY, A CORPORATION OF NEW YORK.

## ELECTRICAL HEATING DEVICE.

1,118,387.

Specification of Letters Patent.

Patented Nov. 24, 1914.

Application filed October 16, 1913. Serial No. 795,559.

*To all whom it may concern:*

Be it known that I, EZECHIEL WEINTRAUB, a citizen of the United States, residing at Lynn, county of Essex, State of Massachusetts, have invented certain new and useful Improvements in Electrical Heating Devices, of which the following is a specification.

The present invention relates to electrical resistances, particularly for furnaces, or other heating devices, and its object is to furnish a resistor of relatively high electrical resistance, which is cheap, rugged and not easily oxidized at a high temperature.

There are at present available for industrial uses, electrical resistance furnaces capable of continuous operation in air at temperatures up to 900° C. For higher temperatures it is necessary to either resort to the very expensive platinum for the resistor, or to surround the heater by a protective atmosphere. For many purposes, particularly in foundries, a simple rugged furnace operable in air at temperatures up to 1300° C. is desired, for example, for melting copper, brass and other metals.

In accordance with my present invention, I have provided an electric furnace having a resistor operable continuously in a furnace in air at temperatures up to 1300° C. and even higher without appreciable oxidation.

My novel resistance unit consists of a refractory core having a rising volt-ampere characteristic, and a surrounding shell of silicon or silicon alloy, the latter as a rule having a negative temperature resistance coefficient and the two elements preferably being proportioned to give the resistor unit as a whole an increasing voltage drop with increasing current.

In the accompanying drawings, Figure 1 shows in perspective a resistance unit with terminals attached; Figs. 2 and 3 are sectional views showing the relative size of the core and the outer shell of silicon, also the structure of the terminal and Fig. 4 illustrates in perspective a furnace containing the novel resistor.

Silicon has a high breakdown characteristic and a high negative temperature coefficient of resistance. Therefore, a voltage high enough to break down the initially high resistance of the silicon is too high for heating a silicon resistor at incandescence. The negative temperature coefficient will cause the

conductivity to progressively increase causing so great a current to flow as to destroy the resistor. This characteristic of silicon would necessitate either operating the silicon resistor in series with large external resistance, thereby causing waste of energy, or operating the resistor from a transformer having two windings and shifting connections from a high voltage winding to a low voltage winding after the furnace has been heated up.

In my new form of resistor this high breakdown resistance is eliminated and a resistor having preferably a rising volt-ampere characteristic is provided through the instrumentality of the core which, being a good conductor, initially acts as a heater for the silicon and also prevents the undue rise of current with a rise of temperature. It is not absolutely necessary that the composite conductor have as a whole an increase in voltage drop with an increase in current over the whole range of operating temperature for even though it should have at a high temperature a slightly drooping characteristic it will require only a very small series resistance in order to prevent an abnormal increase of current and over-heating of the resistor.

In the preferred form of my invention as shown in Figs. 1 and 2, I cast silicon about a core of tungsten although graphite may be used as a core material with almost equal success. The relative size of the core and shell is governed not only by the resistance characteristic of the core but also by other factors such as the heat insulation afforded by the furnace structure. Ordinarily a composite conductor consisting of a tungsten core 1 and a silicon shell 2 which has an outside diameter of about  $\frac{1}{2}$ " will require a core about  $\frac{1}{16}$ " to  $\frac{3}{16}$ " in diameter. The silicon protects the tungsten graphite or the refractory conductor from oxidation as silicon at a high temperature becomes coated with a thin film of protective oxid.

The terminals constitute an important feature in a silicon resistor as the thin film of silica forming on its surface, particularly when cold, has a very high resistance. Mechanically fitting the terminals to the silicon, no matter how well done, will not prevent the formation of this film. I have found that it can be prevented by casting into intimate contact with the silicon a metal

such as copper, aluminum, cupreous alloys or the like.

Claims on a terminal for a silicon resistor are made in my co-pending application, 5 Serial No. 862,339, filed September 18, 1914, as a continuation in part of the present application.

The end of the resistor is preferably left with the core 1 projecting beyond the silicon 10 and is provided with a shell 3 of some suitable refractory metal such as iron or the refractory alloy of chromium, nickel, iron and manganese, known on the market as calorite. Into this cup-shaped shell is cast the metal 15 4 which flows into intimate contact with the silicon as well as with the core. The shell 3 may either be left on the finished resistor or removed as desired.

The resistance rods thus produced may be 20 inserted in slots or grooves upon the inner surface of a fire brick cylinder 5, the terminals projecting beyond the ends of the cylinder. The rods should be flush with the inner surface of the cylinder 5. Inside of 25 the cylinder is fitted a lining 6 which may consist also of fire-brick or other refractory nonconducting material. The rods are all connected in series, for example, by copper straps or flexible strands 7 as indicated, current being supplied by the terminal conductors 8 and 9.

What I claim as new and desire to secure by Letters Patent of the United States, is:—

1. An electric furnace resistor, comprising a core and shell electrically connected in parallel in intimate thermal relation with one another, one of said elements consisting

of silicon and the other of a refractory material having a rising volt-ampere characteristic, said elements being proportioned to 40 give the resistor an increasing voltage drop with increasing current.

2. An electric furnace resistor comprising a core of tungsten and a shell of silicon in close contact therewith. 45

3. An electric furnace resistor comprising a core of tungsten and a shell of silicon in contact therewith, proportioned as to largely reduce the negative temperature resistance coefficient of the silicon. 50

4. An electric heater comprising a core of refractory material having a rising volt-ampere characteristic, and a layer of silicon surrounding the same and electrically in parallel therewith, said core being proportioned to substantially compensate the negative temperature coefficient of the silicon. 55

5. An electric heater comprising a core of refractory material having a rising volt-ampere characteristic and a layer of refractory material operable at a higher temperature in the air having a drooping volt-ampere characteristic surrounding said core and electrically in parallel therewith, said resistance elements being proportioned to 60 have as a whole an increasing voltage drop with increasing current. 65

In witness whereof, I have hereunto set my hand this 9th day of October 1913.

EZECHIEL WEINTRAUB.

Witnesses:

JOHN A. McMANUS, Jr.,  
ROBERT SHAND